

## UNITED STATES PATENT OFFICE

1,969,396

## PRODUCTION OF METALLIC ARTICLES

Franz Duftschmid, Heidelberg, Germany, assignor  
to I. G. Farbenindustrie Aktiengesellschaft,  
Frankfort-on-the-Main, Germany

No Drawing. Application January 5, 1931, Serial  
No. 506,761. In Germany January 17, 1930

10 Claims. (Cl. 29—189)

The present invention relates to improvements in the production of porous or non-porous metallic articles.

5 I have found that porous or non-porous metal articles are obtained in a particularly advantageous manner when several substances in a finely divided state which are capable of being sintered to a coherent mass when in such state, are arranged in a plurality of layers which are 65 different from each other according to their composition, and the whole is then subjected to a sintering treatment by mechanical pressure or heat or both mechanical pressure and heat, but without melting, whereby consolidation of the 70 whole mass to a porous or non-porous article occurs.

The said substances capable of being sintered to a coherent mass may be finely subdivided free 20 metals or metallic compounds which are capable of being converted into the metallic state in which they can be alloyed, or they may be non-metals capable of alloying with the other constituents of the same layer and/or of the adjacent layer or 25 layers. When employing finely divided metals for the said purpose, it is preferable to employ the metals which have been obtained by the 30 thermal decomposition of the corresponding metal carbonyls, because the metals so obtained are particularly suitable for alloying and sintering. Suitable non-metals which may be used according to the present invention are silicon, 35 carbon and arsenic. When employing metal compounds of the aforesaid nature these may be the oxides or other reducible metal compounds, or they may contain the metal in chemical combination 40 with one of the aforesaid non-metals capable of alloying, as is the case for example with the metal carbides. When employing metallic oxides or other reducible metal compounds, it is in most 45 cases necessary to carry out the consolidation by sintering in a reducing atmosphere, but in some cases solid reducing agents present in the mass may be used; thus, when a metallic oxide is present in the mass, the oxygen contained therein 50 may be removed during the consolidation or sintering by interaction with carbon present in the free state or in the form of carbides with the formation of gaseous oxygen compounds of carbon.

The conditions under which the consolidation of sintering is carried out depend of course on the nature of the substances to be combined with each other. In many cases consolidation takes 55 readily place by the application of mechanical pressure alone. In other cases, for example when preparing metallic masses in which one of the components is finely divided steel, the mechanical pressure which would be necessary for consolidation without heat, would be excessively high, and

in such cases it is therefore preferable to effect the consolidation by heat, without melting, and with or without the aid of mechanical pressure. When both heat and mechanical pressure are employed, it is possible first to apply heat 65 and only then mechanical pressure, or mechanical pressure may be applied first and the mass then subjected to the action of heat, or heat and mechanical pressure may be applied simultaneously. 70

The process according to the present invention may be carried out for example by charging different metal powders in the form of layers into moulds and then consolidating them to porous or non-porous metal articles by a treatment by 75 mechanical pressure and/or heat without melting, which may be carried out either simultaneously or in any sequence and for example while heating directly to the desired temperature or by heating in stages and under a constant of gradually increasing mechanical pressure. The pressure treatment may be carried out by the usual methods such as pressing, rolling, or forging, plates, sheets, billets, rods, tubes, wires or other articles thus being obtained. 80

By the process in accordance with the present invention it is possible to prepare metal articles having a composition which varies locally. Thus, metal articles may be prepared in accordance with the present invention, which at different 90 places consist of different metals and/or alloys, as for example articles the surface of which wholly or partly has a composition entirely different from that of the core. Different parts of the surface may also be provided by the process 95 in accordance with the present invention with coatings having different compositions.

A modification of the process in accordance with the present invention consists in first working up the single layers, of which the final article 100 is to be prepared, into porous solid pieces of which each has a uniform composition throughout, but of which all or several have compositions different from those of the others, the porous solid layers then being consolidated and united with 105 each other by a further treatment by mechanical pressure and/or heat into a porous or non-porous metallic article.

The single layers of metal powder may also be worked up each by itself or several together by 110 a treatment by mechanical pressure and/or heat to give porous metal articles, the latter then being combined with layers of finely divided substances capable of alloying with each other or with the said consolidated layers, said layers of 115 finely divided substances having a composition different from that of the consolidated layers, by a further treatment by mechanical pressure and/or heat. The pretreatment of several or all of the layers, whereby these are converted into 120

porous consolidated layers, has the great advantage that the filling of the moulds with the finely divided initial substances is substantially facilitated; thus, it is as a rule rather difficult to arrange in a mould a plurality of vertical layers, each consisting of pulverulent material, vertically one beneath the other. Since large amounts of powder are preferably sintered in moulds having greater dimensions in the vertical direction than in the horizontal, it is preferable to consolidate one or more of the said layers in vertical moulds, whereby the aforesaid difficulties in filling vertical moulds with several different powders are avoided. These partly consolidated layers can then easily be arranged in a mould in any desired position with or without inserting between them layers of pulverulent material, and further consolidated therein by heat and/or mechanical pressure. Another advantage of the pretreatment of several or all of the layers is the fact that it is possible during such preliminary consolidation to employ the conditions which in each case are most favourable for the substance or mixture of substances treated; thus, different layers of different composition may be brought by the preliminary consolidation to a uniform density, whereby the final consolidation is much simplified in that there is no risk that one or more of the individual layers shrink more than the others, whereby they would be destroyed by cracks or would suffer deformation, or that the individual layers do not adhere firmly together due to a different degree of shrinkage.

The importance of the process according to the present invention consists inter alia in the fact that bimetals which hitherto have been prepared by welding together two pieces of metal, are obtained in a simple manner directly from metal powders, and that metal articles having coatings stable to corrosion or heat and of any desired composition can be prepared. It is surprising that such non-uniform articles can be rolled out into sheets without one of the layers tearing or breaking.

It is also possible according to the present invention to prepare metal articles of uniform or substantially uniform composition by subjecting the metal articles to a further heat treatment, following after the first treatment immediately or later, for the purpose of homogenization by diffusion of the constituents of adjacent layers into each other.

The process in accordance with the present invention is also advantageous in that it is possible in the preparation of uniformly composed articles of alloys, for example, to cover a mixture of alloying constituents of the composition of the desired alloy with a layer consisting of the nobler and therefore more difficultly oxidizable alloy component, the mass then being subjected to a consolidating treatment by mechanical pressure and/or heat. In this manner the less noble component in the interior is protected from combustion during the consolidation treatment. If the resulting article then be subjected to a further heat treatment as hereinbefore described, a homogeneous alloy having no injury by combustion or oxidation is obtained. In order to facilitate the production of a substantially uniform article it is preferable to make the outer layer thin in comparison with the core consisting of the less noble component, because in this case diffusion with the formation of a substantially uniform article does not consume so much time. The aforesaid method of working in accordance with the present invention is particularly valua-

ble for making alloys from iron and one or more components which are more readily oxidized than iron, as for example silicon, chromium, manganese or aluminium; the aforesaid disadvantage of combustion or oxidation of the less noble component was particularly troublesome in the methods hitherto known for producing such alloys, and this disadvantage is overcome according to the present invention, even when carrying out the consolidation by the simultaneous employment of both heat and mechanical pressure without excluding air. According to the present invention transformer sheets may be prepared for example by consolidating a mixture of iron powder and silicon powder between thin layers of iron powder in the manner hereinbefore described; by sufficiently extending the heat treatment, the original surface layer free from or poor in silicon may be caused to diffuse with the core of the sheet, so that completely or practically completely homogeneous sheets are produced.

The process according to the present invention is also suitable for the preparation of metal articles having special magnetic properties, for example by working up layers having different ferromagnetic properties into an article of non-uniform composition in the manner hereinbefore described.

The following examples will further illustrate the nature of this invention, but the invention is not restricted thereto.

#### Example 1

A flat, rectangular mould consisting of heat resisting material such as fire-clay, or a chromium nickel alloy or the steel known in the trade as NCT 3 steel of the firm of Krupp, and the inner side of which mould is sprayed with an aqueous suspension of magnesium oxide and then dried, is charged with iron powder obtained by the thermal decomposition of iron carbonyl, until nine tenth of the form are filled. The remaining space is filled with nickel powder obtained by the thermal decomposition of nickel carbonyl. The mould is then heated in an atmosphere of hydrogen first for 12 hours to 650° C. and then for 6 hours to 1100° C. The compounded sintered mass obtained is rolled into plates while warm. An iron plate is obtained which is coated with a homogeneous, tight coating of nickel which adheres well. After pickling and glowing, the plates may be further rolled in the cold and finally worked up by the usual heat treatments such as annealing or glowing. The resulting nickel plated metal can be stamped in a very good manner and may be employed for the manufacture of the most different articles, such as cooking pans or electric fixtures and the like.

#### Example 2

A mould of the kind referred to in Example 1 is filled to one tenth of its height with nickel powder containing carbon, obtained from nickel carbonyl, which is mixed with sufficient nickel oxide for decarbonizing. Iron powder containing carbon, obtained from iron carbonyl, in admixture with iron powder containing oxygen, obtained from iron carbonyl is filled in as the second layer occupying further eight tenths of the height of the mould, and finally a mixture of nickel and nickel oxide similar to the first one is filled in as the upper layer. The mould is provided with a cover and is heated for from 3 to 4 hours to 1200° C. in a reverberatory furnace, whereby carbon monoxide and carbon dioxide are disengaged and a sintered piece is obtained which

consists of three metallic layers connected with each other. The material having a density of about 6 is rolled out in the heat to a sheet nickel-plated on both sides. It may be further worked 5 up as described in the foregoing example.

*Example 3*

Two intimate mixtures of iron powder and nickel powder are prepared, the one containing 10 36 per cent and the other 41 per cent of nickel. The two mixtures are separately filled into a mould, so that two layers of the same thickness each consisting of one of the said mixtures are formed. The mould is then heated to about 15 1300° C. in an atmosphere of hydrogen. The resulting sintered material is then rolled out into plates while still having this temperature. The plates are then heated for six hours to about 20 1200° C. for effecting diffusion within each of the said layers, whereby, however, no substantial diffusion between the two different layers takes place. The plates are then rolled out into sheets at about 1300° C. In this way bi-metal sheets 25 consisting of two different iron nickel alloys, one with 36 and the other with 41 per cent of nickel, are obtained.

*Example 4*

Copper powder is pressed at room temperature 30 into a plate having a specific gravity of 3.5. A layer of iron powder obtained from iron carbonyl of five times the thickness of the copper plate is then arranged on said plate and the mass is heated for five hours to about 800° C. in an atmosphere of hydrogen. A coherent sintered 35 mass composed of two layers is obtained which is rolled out into sheet metal at 850° C. In this way a coppered sheet iron is obtained in which the copper coating has about one fifth of the thickness of the whole sheet.

*Example 5*

Two layers of metallic powders, the one consisting of an intimate mixture of 67 parts of nickel from nickel carbonyl, 28 parts of copper 45 and 5 parts of iron and the other consisting of iron powder without an admixture, are sintered together by heating to about 1000° C. for 10 hours in an atmosphere of hydrogen. The sintered mass is rolled out into sheets at about 1000° C. 50 and the sheets are kept at this temperature for 6 hours. A sheet iron coated on one side with the alloy known in the trade as Monel metal is obtained.

In the appended claims the term "mechanical 55 compression moulding treatment" is meant to comprise such mechanical treatments as forging or rolling in which the material is subjected to the action of mechanical pressure and simultaneously undergoes substantial deformation.

60 In the appended claims wherever a "metal" is referred to, it is to be understood that not only free metals but metal compounds, such as oxides which are capable of being converted into metals under the conditions of working, or metal compounds, such as carbides which are capable of 65 alloying with other metals are contemplated.

What I claim is:—

1. The process of producing metallic articles 70 which comprises arranging a plurality of substances in a finely divided state in adjacent layers of different composition, all of said substances being capable of being sintered to a coherent mass when in a finely divided state and at least one of them being a finely divided metal obtained from the corresponding metal carbonyl,

subjecting said layers of material to a sintering treatment by the action of heat alone and then subjecting the sintered material to a mechanical compression molding treatment.

2. The process according to the preceding 80 claim in which all the substances used are free metals in a finely divided state.

3. The process according to claim 1 in which all the substances used are metals in a finely divided state obtained from the corresponding 85 metal carbonyls.

4. The process of producing metallic bodies 90 which comprises arranging a plurality of finely-divided metals which are capable of being sintered to a coherent mass when in such a finely-divided state, in layers adjacent each other, the metal portion of each layer being different from the metal portion of its adjacent layer and the metal portion of at least one layer being derived from the carbonyl of that metal, and subjecting the mass to a sintering treatment by the action of heat alone.

5. The process defined in the preceding claim 100 in which at least one of the layers is consolidated to a porous mass by a consolidating treatment prior to being arranged adjacent the other layers.

6. The process of producing metallic bodies 105 which comprises arranging a plurality of finely-divided free metals, which are capable of being sintered to a coherent mass when in such a finely-divided state, in layers adjacent each other, the metal of each layer being different from the metal of its adjacent layer and the metal portion of at least one layer being derived from the carbonyl of that metal, and subjecting the mass 110 to a sintering treatment by the action of heat alone.

7. The process of producing metallic bodies 115 which comprises arranging a plurality of finely-divided metals, which are capable of being sintered to a coherent mass when in such a finely-divided state, in layers adjacent each other, the metal portion of each layer being different from the metal portion of its adjacent layer and the metal portion of at least one layer being derived 120 from the carbonyl of that metal, and subjecting the mass to a sintering treatment by the action of heat alone, and then subjecting the sintered material to a mechanical compression moulding treatment.

8. The process of producing metallic bodies 125 which comprises arranging a plurality of finely-divided free metals, which are capable of being sintered to a coherent mass when in such a finely-divided state, in layers adjacent each other, the metal of each layer being different from the metal of its adjacent layer and the metal portion of at least one layer being derived from the carbonyl of that metal and subjecting the mass to a sintering treatment by the action of heat alone, 130 and then subjecting the sintered material to a mechanical compression moulding treatment.

9. The process of producing metallic bodies 135 which comprises arranging a layer of finely-divided nickel derived from nickel carbonyl adjacent a layer of finely-divided iron from iron carbonyl and sintering the mass by the application of heat alone.

10. The process of producing metallic bodies 140 which comprises arranging a layer of finely-divided copper adjacent a layer of finely-divided iron from iron carbonyl and sintering the mass by the application of heat alone.